

# United States Patent

[11] 3,615,570

[72] Inventors **Georg Werner;  
Herbert Rauhut, both of Wiesbaden-  
Biebrich, Germany**  
[21] Appl. No. **529,650**  
[22] Filed **Feb. 24, 1966**  
[45] Patented **Oct. 26, 1971**  
[73] Assignee **Keuffel & Esser Company  
Morristown, N.J.**  
[32] Priority **Feb. 24, 1965**  
[33] **Germany**  
[31] **K 55375**

[54] **DIAZO-3-TRIFLUOROMETHYL-4-  
TERTIARYAMINOBENZENE COMPOUNDS**  
7 Claims, No Drawings

[52] U.S. Cl. .... **96/91 R,  
96/49, 96/75, 260/141, 260/142, 260/247.5 R,  
260/293 D, 260/326.85, 260/570.5 R**  
[51] Int. Cl. .... **C07c113/00,  
C07d 29/00, G03c 1/52**  
[50] Field of Search..... **96/49, 75,  
91; 260/141, 142, 326.85, 293 D, 247.5 R**

| [56]                  | References Cited |                        |           |
|-----------------------|------------------|------------------------|-----------|
| UNITED STATES PATENTS |                  |                        |           |
| 2,350,843             | 6/1944           | Vanselow et al.....    | 96/91     |
| 2,298,444             | 10/1942          | Weissberger et al..... | 96/91     |
| 2,552,354             | 5/1951           | Von Glahn et al.....   | 96/91     |
| 2,793,118             | 5/1957           | Sanders et al.....     | 96/75 X   |
| 3,218,300             | 11/1965          | Kullmar et al. ....    | 260/141 X |
| 3,251,889             | 5/1966           | Kulka.....             | 260/141 X |
| 3,357,968             | 12/1967          | Wilbert et al. ....    | 260/141 X |
| FOREIGN PATENTS       |                  |                        |           |
| 895,250               | 5/1962           | Great Britain.....     | 96/91     |
| 957,838               | 5/1964           | Great Britain.....     | 96/91     |

Primary Examiner—Floyd D. Higel  
Attorneys—J. Russell Juten, Peter F. Willig and Milford A. Juten

**ABSTRACT:** Improved light sensitivity and dye forming coupling speed are obtained in one-component diazo-type copying material useful in preparing intermediate diazo-type reproducible copies through the use as the light-sensitive component a 1-diazo-3-trifluoromethyl-4-tertiary-amin.o-benzene compound.

**1  
DIAZO-3-TRIFLUOROMETHYL-4.  
TERTIARYAMINOBENZENE COMPOUNDS**

In diazotype processes there are already used, as so-called one-component papers for the semiwet development process, diazotype papers which contain, as light-sensitive substance in their reproduction coatings, compounds corresponding to the general formula I



In this formula I, R<sub>1</sub> and R<sub>2</sub> stand for alkyl, aralkyl or cycloalkyl, R<sub>3</sub> for hydrogen or halogen atom, and X for an anion.

These diazo compounds, when developed with one of the usual developers having pH values of 8 to 10 and containing phloroglucinol or resorcinol as coupling components, generally yield brown azo dyes when R<sub>3</sub> in Formula I is halogen, and black azo dyes when R<sub>3</sub> is hydrogen and R<sub>2</sub> is aralkyl.

The alkaline developers which contain polyvalent phenols as coupling components having the disadvantage that they do not keep for long because oxidation by the air sets in. For this reason, in recent times, developers are used having pH values below 8 which correspond to neutral or, preferably, acid reaction, and containing polyvalent phenols as coupling components.

For the successful use of acid developers, diazo compounds with great coupling activity are necessary. As such, compounds of formula II as known:



In this formula II, R<sub>4</sub> stands for a phenylacetamido, thiophenylacetamido, benzoylacetoamido-arylmercapto, alkoxyphenyl or benzoylamino group, and R<sub>5</sub> and R<sub>6</sub> stand for alkyl, aralkyl or aryl.

The coupling dyes which are achieved with acid developers in combination with the diazo compounds of formula II are in general of black colors and those achieved in combination with the rapid-coupling compounds of formula I are of violet hues. In fact, the commercially available diazo-type papers for acid development do only give copies with black or with violet lines. For this reason, diazo compounds which, when developed with acid developers, yield colors other than those mentioned above, are of great interest for practical purposes. The reason for this is not only that the consumer is accustomed for example to brown lines from alkaline development, but also because brown dyes on transparent supports absorb ultraviolet light particularly well.

It was now found that with diazotype material which contains, as light-sensitive substance in the reproduction coating, a diazo compound corresponding to the general formula III



(III)

wherein R<sub>1</sub> and R<sub>2</sub> stand for alkyl, aralkyl or cycloalkyl groups which may be substituted or not, or R<sub>1</sub> and R<sub>2</sub> together with the nitrogen form a heterocyclic ring, and X is an anion, red-brown to brown-red, even brown-orange, coupling dyes of excellent covering power are obtained when acid developers are used. The diazo compounds according to formula III are distinguished by very great coupling activity, which is of advantage also when alkaline developers are used.

- 10 The diazo compounds of formula I, named in British Pat. specification No. 711,380 among others, wherein an alkyl group stands for R<sub>3</sub>, do, after exposure of the reproduction coating sensitized with them, also yield images with brown hues when acid developers are used. However, their coupling activity and the covering power of the coupling dyes is lower than in the case of the corresponding compounds of formula III with a CF<sub>3</sub> group in place of R<sub>3</sub>.

- 15 In German Pat. No. 1,015,679, among other compounds, the chlorostannate of 1-diazo-4-monocyclohexylamino-3-trifluoromethyl-benzene is mentioned. This compound, as a secondary amino diazo compound, is not so light sensitive as the diazo compounds of formula III which bear a tertiary amino group in p-position to the diazo group. Moreover, when development is effected with acid developers, it gives violet-black hues which do not cover so well.

20 The diazo compounds according to formula III may be prepared according to various methods. Their synthesis is particularly simple when a process is used which is another object of the present invention. In this process, 2-chloro-5-nitro-1-trifluoromethylbenzene is used as starting material and this is reacted with a secondary amine of the formula NHR<sub>1</sub>R<sub>2</sub>, wherein R<sub>1</sub> and R<sub>2</sub> have the meaning given above, for example dimethylamine, diethylamine, diisopropylamine-di-n-butylamine, hydroxyethylpropylamine, methylbenzylamine,

25 hydroxyethylbenzylamine, methylcyclohexylamine, pyrrolidine, morpholine, thiomorpholine, piperidine, N-alkylpiperazine, N-acylpiperazine. In the case of the secondary amines used for the reaction, the alkyl, cycloalkyl and aralkyl groups or the heterocyclic ring may bear substituents which behave inert in the reaction. The nitro group of the resulting

30 nitroaminotrifluoromethylbenzene with a tertiary amino group is then reduced to the amino group, the amino group is diazotized according to known methods, the anion X is added 35 in the form of a soluble compound comprising the anion X, and in an amount sufficient to precipitate at least part of the formed diazonium compound as a salt of the above formula. Finally, the precipitated salt is separated from the remainder of the reaction mixture.

40 45 The diazo compounds obtained after diazotation may be separated in the form of the chlorides as double salts with zinc chloride, cadmium chloride, stannic chloride, or as sulfates, borofluorides, hexafluorophosphates. The form in which the compound is present after separation has little influence on

50 55 the property of the diazo compound. The diazo compounds according to formula III have good compatibility with the stabilizing agents usual in sensitizing solutions, such as 1,3,6- or 1,3,7-naphthalenetrisulfonic acid, boric acid, tartaric acid, citric acid, and others.

60 As support materials for the diazo reproduction coating according to the invention, photocopying base paper, precoated photocopying base paper, transparent paper, transparentized paper, transparent paper provided with a coating of cellulose acetate which has been made hydrophilic, plastics films, e.g.

65 polyester films or polycarbonate films, suitably pretreated for use as diazotype coating supports, can be used. Diazotype material which contains a diazo compound of formula III as light-sensitive substance in the reproduction coating, cannot only be used with acid developers but can also be developed in 70 alkaline manner. The hues achieved are in general light brown to yellowish brown.

Diazo compounds according to formula III, whose coupling intensity is less great, can also be used for the preparation of so-called two-component diazotype material. Depending on the nature of the coupling component used together with

them, which must, of course, have little coupling activity, different hues can be achieved by development with ammonia vapor.

In the following examples, parts by volume bear the same relation to parts by weight as cc. to g.

#### EXAMPLE 1

As base paper suitable for the preparation of diazo-type material and which had previously been provided with a precoat of colloidal silicic acid and polyvinyl acetate was coated on the precoated side with a solution which contained in 1,000 parts by volume of water:

- 5.0 parts by weight of citric acid
- 36.0 parts by weight of sodium naphthalene-1,3,6-trisulfonate,
- 0.5 parts by weight of saponine
- 50.0 parts by volume of isopropanol
- 26.0 parts by weight of the diazo compound from 1-amino-4-methylbenzylamino-3-trifluoro-methylbenzene as borofluoride.

After drying of the applied solution, the sensitized paper was image-wise exposed under a transparent original and developed with a solution which in 1,000 parts by volume of water contained:

- 3.0 parts by weight of phloroglucinol
- 96.0 parts by weight of trisodium citrate
- 24.2 parts by weight of sodium benzoate
- 19.7 parts by weight of adipic acid
- 57.0 parts by weight of sodium chloride
- 2.0 parts by weight of sodium salt of alkylnaphthalenesulfonic acid, e.g. the product marketed under the trademark Nekal A.

The pH value of the developer is 6. Brown images on a white background were obtained.

When, instead of the diazo compound used above, there was used in the sensitizing solution the diazo compound from 1-amino-4-methylbenzylamino-3-methylbenzene, violet images on a white background were obtained. After application of the developer, the violet coupling dye was formed but distinctly more slowly than when the diazotype material according to the invention was used.

#### EXAMPLE 2

Transparent paper which is coated on one side with a partially saponified cellulose acetate coating was coated on the precoated side with the sensitizing solution described in example 1, exposed under a line original after drying, and treated as in example 1. Brown-red lines with good covering power were obtained. In this case, too, the dye formed very rapidly directly after application of the developer.

#### EXAMPLE 3

Base paper without a precoat and which is suitable as coating support for the preparation of diazotype material, was coated with a solution which contained in 1,000 parts by volume of water:

- 5.0 parts by weight of citric acid
- 36.0 parts by weight of sodium naphthalene-1,3,6-trisulfonate
- 50.0 parts by volume of isopropanol
- 25.0 parts by volume of triglycol
- 1.0 part by weight of saponine
- 25.0 parts by weight of the diazo compound from 1-amino-4-piperidino-3-trifluoromethyl-benzene as borofluoride.

After drying of the applied solution, the sensitized base paper was image-wise exposed under a transparent line original and developed with a solution which, in 1,000 parts by volume of water, contained the following substances and had a pH value of 6.3:

- 57.0 parts by weight of potassium adipate
- 23.0 parts by weight of sodium benzoate
- 1.0 part by weight of adipic acid
- 5.0 parts by weight of thiourea

5.0 parts by weight of cane sugar

6.5 parts by weight of phloroglucinol

4.0 parts by weight of resorcinol

2.0 parts by weight of sodium salt of alkylnaphthalenesulfonic acid, e.g. the product marketed under the trademark Nekal A.

Copies with red-brown lines on a white background were obtained.

When the sensitized paper was developed with a solution which contained in 1,000 parts by volume of water:

20.0 parts by weight of borax

20.0 parts by weight of trisodium phosphate

40.0 parts by weight of trisodium citrate

6.0 parts by weight of resorcinol

6.0 parts by weight of phloroglucinol

30.0 parts by weight of thiourea

2.0 parts by weight of the sodium salt of alkyl-naphthalenesulfonic acid, e.g. the product marketed under the trademark Nekal A.

Copies in neutral brown hues on a white background were obtained.

When the diazo compound from 1-amino-4-morpholino-3-trifluoromethylbenzene was used as light-sensitive substance in the reproduction coating of the diazotype paper, under the same conditions, with the two developers mentioned above, copies with yellowish hues were obtained.

#### EXAMPLE 4

30 An already precoated diazotype base paper of the type mentioned in example 1 was coated on the precoated side with a solution which contained in 1,000 parts by volume of water:

40.0 parts by weight of citric acid

40.0 parts by weight of thiourea

26.0 parts by weight of 7-hydroxynaphthimidazole-1,2

50.0 parts by volume of isopropanol

25.0 parts by volume of triglycol

20.0 parts by volume of glacial acetic acid

38.5 parts by weight of diazo compound from 1-amino-4-pyrrolidino-3-trifluoromethyl-benzene as zinc chloride double salt.

After drying of the applied solution, the thus obtained sensitized paper was image-wise exposed under a transparent line original and developed with ammonia vapor. Copies with red-brown lines on a white background were obtained.

The table following the next paragraph gives several representative diazo compounds according to formula III.

It is apparent that the described examples are capable of many variations and modifications within the scope of the present invention. All such variations and modifications are to be included within the scope of the present invention.

| $\begin{array}{c} R_1 \\ \backslash \\ N \\ / \\ R_2 \end{array}$ | $X$ | Melting point<br>of the corre-<br>sponding nitro<br>compound,<br>°C. |
|-------------------------------------------------------------------|-----|----------------------------------------------------------------------|
|-------------------------------------------------------------------|-----|----------------------------------------------------------------------|

| $\begin{array}{c} R_1 \\ \backslash \\ N \\ / \\ R_2 \end{array}$ | $\begin{array}{c} CF_3 \\    \\ N \\    \\ CF_3 \end{array}$ | Melting point<br>of the corre-<br>sponding nitro<br>compound,<br>°C. |
|-------------------------------------------------------------------|--------------------------------------------------------------|----------------------------------------------------------------------|
|-------------------------------------------------------------------|--------------------------------------------------------------|----------------------------------------------------------------------|

| $\begin{array}{c} R_1 \\ \backslash \\ N \\ / \\ CH_3 \end{array}$ | $\begin{array}{c} CH_3 \\    \\ N \\    \\ CH_3 \end{array}$ | $\begin{array}{c} Cl \\    \\ ZnCl_2 \\ / \\ \backslash \\ Cl \\    \\ CdCl_2 \end{array}$ | 48 |
|--------------------------------------------------------------------|--------------------------------------------------------------|--------------------------------------------------------------------------------------------|----|
|--------------------------------------------------------------------|--------------------------------------------------------------|--------------------------------------------------------------------------------------------|----|



<sup>1</sup> Melting point of the corresponding amino compound.

What is claimed is:

1. Diazotype material comprising a support bearing a composition comprising a light-sensitive diazo compound corresponding to the general formula



- 62-63 10 wherein R<sub>1</sub> and R<sub>2</sub> are selected from the group consisting of lower alkyl, hydroxy alkyl, aralkyl, cyclohexyl radicals, and heterocyclic radicals in which R<sub>1</sub>, R<sub>2</sub> and the nitrogen atom form 5- or 6-membered nitrogen-containing heterocyclic radicals, and X stands for an anion.
- 15 2. Diazotype material according to claim 1 wherein said diazo compound is 1-diazo-4-methylbenzylamino-3-trifluoromethylbenzene-diazonium borofluoride.
3. Diazotype material according to claim 1 wherein said diazo compound is 1-diazo-4-piperidino-3-trifluoromethylbenzene diazonium borofluoride.
4. Diazotype material according to claim 1 wherein said diazo compound is 1-diazo-4-morpholino-3-trifluoromethylbenzyl diazonium borofluoride.
5. Diazotype material according to claim 1 wherein said diazo compound is 1-diazo-4-pyrrolidino-3-trifluoromethylbenzyl diazonium zinc chloride.
6. Diazo compound corresponding to the general formula



wherein R<sub>1</sub> and R<sub>2</sub> are selected from the group consisting of lower alkyl, hydroxy alkyl, aralkyl, cyclohexyl radicals, and heterocyclic radicals in which R<sub>1</sub>, R<sub>2</sub> and the nitrogen atom form 5- or 6-membered nitrogen-containing heterocyclic radicals, and heterocyclic radicals, and X stands for an anion.

7. 4(N-pyrrolidino)-3-trifluoro methyl aniline.

\* \* \* \* \*